# EUROPEAN PATENT SPECIFICATION

(11) **EP 0 731 738 B1**
(45) Date of publication and mention of the grant of the patent: **06.06.2001**
(21) Application number: 95904223.5
(22) Date of filing: 30.11.1994
(51) Int. Cl.: B32B 15/08, B32B 7/12, B21D 51/26

(54) **DRAWN AND IRONED CANS OF A METAL-PLASTIC CONSTRUCTION AND THEIR FABRICATION PROCESS**
TIEFGEZOGENER UND ABGESTRECKTER BEHÄLTER VON METALLKUNSTOFF UND IHREN HERSTELLUNGSVERFAHREN
BOITES EMBOUTIES/ETIREES DE STRUCTURE METALLOPLASTIQUE ET LEUR PROCEDE DE FABRICATION

(30) Priority: 01.12.1993 FR 9314619
(43) Date of publication of application: 18.09.1996
(73) Proprietor: McHenry, Robert J., St.Charles, IL 60174 (US)
(72) Inventor: McHENRY, Robert, J., St. Charles, IL 60174 (US); PETIT, Dominique, F-38340 Pommiers-la-Placette (FR)
(74) Representative: Becker Kurig Straus
(86) International application number: US9413922
(87) International publication number: WO9515226

(56) References cited:
- EP-A- 0 034 781
- EP-A- 0 046 444
- EP-A- 0 115 103
- EP-A- 0 134 958
- WO-A-82/00020
- GB-A- 2 237 763
- US-A- 3 760 751
- US-A- 5 181 409
- US-A- 5 193 265
- IRON & STEEL, vol. 26, no. 2, February 1953, GUILDFORD; GB, pages 63-66, XP000579822 S.Y. CHUNG ET AL.: "CYLINDRICAL SHELLS. AN EXPERIMENTAL INVESTIGATION INTO REDRAWING"

## Description

### Background of the Invention

The present invention generally relates to fabrication, by drawing and ironing, of cans for use in packaging of beverages or foods and containers for aerosols. More precisely, the present invention relates to new and improved metal-plastic laminate construction of the type including metal-polymer-metal, that is in which a layer of polymer is interposed between two metal sheets to which it is adhered.

Hereinafter, the terms metal-plastic-metal, metal-polymer-metal, or more simply the abbreviation MPM are used without particular distinction to identify the new and improved laminar materials of the present invention.

There are numerous documents describing layered metal-plastic constructions. The majority of these concern metal-polymer or poly-metal-polymer constructions, metal-polymer-metal constructions being rarer.

Of these documents that do mention MPM constructions, none teaches any preferred range of materials and thicknesses which are specially suitable for making drawn and ironed beverage or food cans.

By way of illustration, WO 82/00020, published on January 7, 1982, describes a metal-plastic construction which in its simplest form includes a polyethylene (PE) film attached to a foil or plate of metal. Another embodiment includes two films of PE attached to opposite surfaces of a metal plate to form a complex, PE-metal-PE. Finally, a third embodiment consists of two plates or foils of metals attached to opposite surfaces of a PE film. The PE used, obtained by copolymerization under a low pressure of ethylene and of butene-1, is of a linear low density type (LLDPE) having a density of between 0.91 and 0.94. The LLDPE described in this application, has the interesting property of adhering directly to the metal without needing to use an adhesive. It suffices to adhere it to the metal by the simultaneous application of heat and pressure (heat sealing).

The metallic substrates described in this application include: steel, steel having a coating of tin or of chrome or of chrome/oxide or of zinc, aluminum treated or not with nickel, copper, or zinc. It may have undergone a chemical conversion treatment.

Although there is no explicit teaching as to the desired absolute or relative examples of simple metal-plastic constructions, the published application describes films of different types of polyethylene of 100 µm (microns) thickness that are heat sealed onto the plates of different metals, such as steel, tin-plated steel, steel coated with chrome-chrome oxide, or aluminum of a thickness of 210 µm (microns). The specimens obtained are then formed into hollow articles by folding, stamping, drawing, wall-ironing. The adhesion of the coatings is compared and demonstrates the superiority of linear low density polyethylene (LLDPE).

The French patent No. FR2 665 887 (Pechiney Emballage Alimentaire) describes a capsule to fit over a cork made by drawing, drawing and ironing, or flow turning, characterized in that it is comprised of two layers of aluminum bound together by an adhesive layer of Shore hardness less than 80. The adhesive layer can be constituted of an ethylene acrylic acid or of polyethylene, or of polypropylene modified with acid functionality. The total thickness of the complex is comprised between 120 and 400 µm (microns) with the following percentage distribution of the total thickness:

| | |
|---|---|
| Outer layer of aluminum | 20 to 50% |
| Adhesive layer | 3 to 30% |
| Inner layer of aluminum | 40 to 60% |

European Patent Application EP-A-0 046 444 assigned to Schwerzerische Aluminum AG describes an MPM composite laminate foil in which the plastic layer could be as thick as the two metal layers combined. One stated requirement for achieving deep drawability is to select the plastic core layer and the metal surface layers such that when the composite is elongated, the load borne by the plastic core is greater than that borne by each of the metal strips. This condition is achieved by use of an oriented or stretched plastic layer. It is also stated that the soft or half-hard aluminum thin strip is particularly well suited. There is no teaching of drawing and ironing as a suitable process, but rather deep drawing and deep drawing by elongation, which are the conventional processes for such semi-rigid containers.

A similar approach to MPM constructions is described in European Patent Application EP-A-O 034 781 which is assigned to BASF Aktiengesellschaft. The inventors of that application roll the plastic film before combining it with the metal foil in order to give the plastic ductility properties which are more like selected metals.

A metal-plastic-metal structural laminate which can be formed into various useful articles is described in European Application EP-A-0134958 assigned to Dow Chemical Company. This invention is in part defined by a very wide range of thicknesses of the individual layers, of total thicknesses, and of ratio of thicknesses. It is further defined in terms of an ability of the laminate to withstand at least a certain level of stretch formability as measured in a standard laboratory test, the ability to be bent to a given sharp radius without metal rupture, and a certain level of thermal stability.

The patent does not contain any reference to any drawn or drawn and ironed shapes nor to the ability of these laminate constructions to be formed by either a drawing process or by a drawing and ironing process. The laboratory test described is a form of biaxial tension test in which the material is uniformly stretched while maintaining the periphery, fixed in such a way as to thin the material. While such a stretch forming process is conventionally used in forming shallow parts such as automotive panels, it is not used for making food or beverage cans. A conventional drawing process such as is used to make food cans or for the initial steps to make beverage cans allows the material to flow from the periphery and results in little or no thickness reduction.

U.S. Patent 3298559, assigned to Continental Can Company, describes laminated metal-plastic containers, such as cake pans, which are cold drawn in conventional forming dies. Among the metal-plastic containers described are some which are of the MPM type. Although wide ranges of thicknesses of metal and of plastic are claimed, there is no teaching as to the importance of the ratio of these thicknesses. Those examples which cover MPM constructions have a ratio of plastic to total metal thickness of between 5 and 9. The metal layers in the MPM examples are described as dead-soft or zero temper. There is no indication that such containers can be formed by a drawing and ironing process or that drawn containers suitable for food cans can be made.

### Problem Posed

The problem presented to the inventors was that of the improvement of a can for gaseous beverages. Of a capacity in general of around 33 centiliters, of a cylindrical shape, this can is closed by an easy open end, coated internally by a food approved varnish and externally by one or several decorative layers indicating the nature and the brand of the product contained. These coatings are in general applied after the forming of the can.

The most frequently used forming process of these cans is the process of drawing and ironing. This process permits very rapid production cycles, which has permitted the enormous worldwide diffusion of this type of can.

This process, well known to one skilled in the art, is comprised as its name indicates by a first series of one or several passes of drawing and second series of one or several passes of ironing. One starts with a flat circular disc of steel or aluminum alloy of a thickness of around 300 µm (microns). This disc is first drawn for forming an initial shallow cup with the aid of an apparatus represented by Figure la. The initially flat disc (1) is shown there in the course of deformation. It is pressed between a fixed die plate (2) and a pressure plate (3). The descent of the punch (4) driven by a piston permits the formation of the cup which undergoes practically no decrease in thickness. The cup is then formed by a second drawing pass (Figure 1b) where the designating numerals correspond to the same elements as on Figure 1a.

The walls of this cup are then ironed by the aid of a series of ironing rings, generally three in number, of decreasing internal diameter. Figure 2 represents one of these ironing rings and illustrates its functioning. The cup (5) is fit with a slight play on the punch (6) which causes it to penetrate the interior of the ring (7) of which the interior diameter is inferior to the exterior diameter of the cup. This results in a thinning and a corresponding elongation of the wall. The magnitude of the elongation or ironing is regulated by the difference between the exterior diameter of the cup and the interior diameter of the ring. The capacity for deformation of the cup not permitting reaching the final height of the can in a single ironing pass, it is usual as indicated above to place three rings in series passed successively by the cup with the same punch stroke.

Among the elements of cost of the beverage can made by the process reviewed above, the cost of the metal, despite it slight weight, constitutes a preponderant portion. The idea had therefore occurred to the researchers of replacing a part of the metal by a less costly material: plastic.

The modulus of elasticity and the elastic limit of most plastic materials being much less than those of metals, the substitution of plastic for metal faces several structural problems. In addition to these structural problems, there are process problems tied to the fact that metal cans are generally fabricated under conditions considerably different from those used for forming plastics. For example, metal containers are normally fabricated at high speed and at ambient or moderate temperatures, whereas the behavior of plastics is such that plastic containers are fabricated normally at lower speed and at higher temperatures.

Previous researchers, in particular as described in WO82/00020, have shown that thin layers of plastic adhering well to a metal foil are able to be formed by simple modifications to the conventional metal forming processes. This can be explained by the fact that the behavior of the metal-plastic construction during forming is controlled by the stronger and thicker metal and by the fact that the stresses generated in the thin plastic layer or layers are easily transferred to the metal foil as a result of their good adherence.

This restriction to relatively thin plastic layers has not been a problem in the previous research because the role of the plastic was in general to protect the metal against corrosion and that a relatively thin layer of plastic suffices for that protection.

Even though WO 82/00020 states that if desired, the laminates may be made with sheet metal or foil bonded to opposed surfaces of the polyethylene film, there is no indication that thicker plastic layers would be desired or possible in such MPM structures. If one constructed MPM structures using the 100 µm (micron) plastic film and two metal foils of 210 µm (microns) which are described in that patent, the ratio of plastic core thickness to total metal thickness would be less than 0.24. This low ratio, as will be shown, is below that required for the desired cost savings.

In addition to the use of layers of plastic which are thin enough to be dominated in forming by the metal, previous investigators have used two approaches. The first which is illustrated in French Patent FR1414475 and U.S. Patent 4390489 is to carry out the forming starting from a heated material as would be used in conventional plastics processes such as thermoforming.

The second approach is to work with metal-plastic constructions in which the respective materials are selected in such a way that the plastic core dominates the forming and the aluminum deformation follows the deformation of the plastic. In EP-A-o 046 444 described previously, this condition is specified in terms of the load borne by the plastic core being greater than that borne by each of the metal strips. This is achieved by use of soft or half-hard aluminum strip and the use of an oriented or stretched plastic layer.

In EP-A-0 034 781, the inventors cold roll the plastic film in order to make it even more dominant compared to a given metal foil. This enables them to use a somewhat stronger metal foil. Although the inventors do not state their results in terms of the percentage of load which is borne by the metal, that percentage can easily be calculated for each of the layered constructions shown in the example under the assumption that the ultimate metal stress if equal to that of the metal foil when tested by itself. This calculation shows that the metal would bear only 16.4% of the tensile load in the construction which uses the cold rolled film and 20.8% in the comparison sample using a thicker layer of the same plastic film without cold rolling. Here too, there is no mention of drawn and ironed containers nor of the ability of the layer construction to undergo successfully the wall ironing process.

In U.S. Patent 3298559, the inventors do not cold roll or otherwise orient the plastic but in each of the MPM examples given, they do specify that the aluminum foils are dead-soft or zero temper. In addition, the ratio of plastic thickness to total metal thickness is at least 5 to 1 in each MPM example. Although the inventors do not state the percentage of load taken by the metal nor provide mechanical data from which it can be calculated, this combination of dead-soft aluminum and high plastic to metal thickness ratio dictates that the plastic layer will dominate the forming process.

As will be shown below, the use of soft metal alloys or of a layer of plastic which is very thin compared to the total metal thickness would not meet the objective of the present inventors in providing a major reduction in material cost for a container which must resist, at some point in time, an internal pressure or other significant mechanical load.

The current inventors have also found that an unoriented plastic core layer is preferred over an oriented plastic core in terms of the ability to withstand the deeper draws and, in particular, to withstand the subsequent ironing steps required for drawn and ironed beverage and food cans.

To attain the objective of the present invention which is to reduce the thickness and, therefore, the cost of the metal used, the inventors have found that the plastic layer ought to be placed between two metal layers and ought to be thicker than those attained up until now in the containers made of metal-plastic constructions. It is known in other types of mechanical structures to use a low cost or low density material as a central layer placed between two outside layers made from a stronger and more rigid material. Such "sandwich structures are known for achieving a bending resistance approaching that of a single layer of the more solid material of the same thickness as the total thickness of the sandwich.

Even though the less resistant central material contributes to the bending resistance of the structure, it barely contributes to the tensile resistance of the sandwich. This limits the possible reduction of the total thickness of the two external metal layers. The tensile resistance of a structure with relatively thin metal walls such as a container is called membrane strength.

The inventors have found that the pressure at which the base of a rigid container such as a gaseous beverage can start to pass from a concave shape, viewed from the exterior, to a convex shape depends on a complex function of the bending resistance and the membrane strength. This pressure is commonly called bottom buckling pressure. The form of this function of the two types of resistance depends on the exact shape of the concave dome and of the shape of the part of the base which connects the dome to the bottom of the container's wall.

The bottom buckling pressure (P) can be expressed for single layer metal as a function of the thickness by the formula:${\text{P = ke}}^{\text{n}}$ with k = proportionality constant depending on the material, e = thickness of the material, n = exponent varying between 1 and 2 depending on the geometry of the base. When the exponent n is close to 1, this signifies that the buckling pressure is more sensitive to the membrane resistance; when the exponent is close to 2, this signifies that the bottom buckling pressure is more sensitive to the bending resistance. For most beverage can bases, the exponent lies between 1.2 and 1.9. The closer the exponent is to 2, the less thickness of plastic is required for a given thickness of the external metal layers.

Figure 3 shows the plastic thickness eₚ required for a total thickness of the two metal layers eₙ to obtain the same buckling pressure as with an entirely metallic structure with a thickness of 330 µm (microns). As one can observe on the different curves, one needs much less thickness of plastic in the case of an exponent n = 1.7 for which the bending resistance is the most critical than in the case of an exponent n = 1.2, for which the membrane strength is the most critical.

One can see also on this Figure 3 that for a given base configuration and, therefore, for a given value of n, there exists a series of plastic thicknesses eₚ and corresponding total thicknesses of the two metal layers eₘ, which will give the required bottom buckling strength. For a configuration with an exponent of 1.5 for example, all the acceptable combinations correspond to the abscissa and the ordinate of each point of the curve designated 1.5.

In general, the points to the left on each curve represent the most economic structures because they incorporate less of the costly metal and more of the low cost plastic.

One should also note that these points have a ratio of the thickness of the plastic to the total thickness of the metal higher than that which has been realized in the prior art.

It was expected that the fabrication, starting with a MPM structure, of containers with the conventional metal forming processes such as drawing and ironing would be relatively more difficult with structures comprised of less metal and more plastic. One reason for this expectation was that, as much during the drawing as the ironing, the MPM structure is submitted to tensile stresses and one would think, according to the existing technology, that the elongation to rupture of the MPM structure would be the same as that of an entirely metal structure. At this elongation, the plastic material, as a result of its low modulus would support a minor portion of the tensile stresses induced by the drawing and ironing. In order to test the commonly accepted assumption of an equal elongation to rupture, the inventors have done uniaxial tensile tests on several structures with varying thickness of plastic and a constant thickness of 100 µm (microns) for each layer of the exterior aluminum alloy.

They have been surprised to observe that, as shown on Figure 4, the elongation to rupture increased with the thickness of the plastic and attained a maximum in the neighborhood of 300 µm (microns) of plastic, that is a ratio P/(Mᵢ + Mₑ) of 1.5.

Although the explanation of this surprising increase in the elongation to rupture is not perfectly clear, the examination of the specimens after rupture shows that it is related to the ability of the plastic to spread the concentration of stresses resulting from the initiation of necking of one of the external metal layers. The plastic distributes the stresses over a large surface of the opposing external layer, thus preventing the necking of the first external layer from propagating to rupture. If the layer of plastic is relatively thin, this concentration of stresses is transferred to a relatively small surface of the opposite external layer which leads to a simultaneous necking of the two layers. If the layer of plastic is thicker than the optimum value, it seems that the plastic is less capable of transferring the stress concentration to the opposite external layer, and the necking proceeds in a sequential fashion in the two metal layers.

The improvement of the toughness of the MPM constructions characterized by their elongation to rupture has permitted successful drawing and ironing MPM structures with relative thicknesses of plastic significantly higher than had ever been achieved. As indicated above, the economic balance for a given bottom buckling pressure is significantly more favorable with such higher thickness of plastic.

Using data from the same tensile specimens as used to produce Figure 4 in which each metal foil had a thickness of 100 microns and was aluminum alloy 3003 with a tensile rupture strength of 239 MPₐ, the inventors calculated the portion of the total load which was borne by the metal foil. The percentages varied from 99% with a 55 µm (micron) thick core to 82% with a 420 µm (micron) thick core.

### Summary of the Invention

In accordance with these and other objects, the present invention provides new and improved metal-polymer-metal laminates and constructions useful for forming can bodies and cans. The nature and the thicknesses of the layers of the laminate are specially adapted to provide the mechanical characteristics demanded of the metal cans intended, in particular, for the packaging of gaseous beverages or food, as well as, to their means of forming by drawing and ironing.

The present invention has equally as objective a process for the fabrication of metal cans intended for the packaging of food products or of beverages by drawing and ironing of metal-plastic constructions of the type MPM.

### Brief Description of the Drawings

Figures 1a and 1b schematically represent two drawing passes of a circular disc according to the prior art;
Figure 2 represents ironing of the wall of a drawn cup for making it into a can;
Figure 3 represents isobars for the bottom buckling pressure P, the total thickness of the metal eₘ being the abscissa and the thickness of the intermediate polymer layer eₚ being the ordinate;
Figure 4 represents the variation of the elongation to rupture of an MPM construction in which each of the external metal foils has a thickness of 100 µm (microns), as a function of the thickness of the central layer of polymer;
Figures 5a and 5b represent two preferred forms of the base of the punch according to the invention; and
Figure 6 represents mold components for the second drawing pass according to the invention.

### Description of the Preferred Embodiments

Can bodies composed of a base and of a wall in which the generatrice are perpendicular to the base of a metal-plastic construction of the type metal-polymer-metal intended to contain in particular beverages and objects of the invention are characterized in that the metal-plastic construction comprises a central layer of thermoplastic polymer of thickness P coated on its interior and exterior faces with metal foils of respective thicknesses Mᵢ and Mₑ such that the ratio P/(Mᵢ + Mₑ) is superior to 0.5 and that the bodies being fabricated by drawing and ironing, their wall is thinned with respect to the bottom of the can body.

Following the same line of explanation of the problem developed above, this ratio P/(Mᵢ + Mₑ) will be preferably between 0.7 and 2.5 and most preferably between 1 and 2.

In an advantageous method of realization of the metal-plastic construction, the central polymer layer has a thickness before ironing between 100 and 500 µm (microns), each of the metal foils a thickness between 25 and 150 µm (microns) before ironing. These thicknesses are evidently less in the thinned walls of the body. In a further advantageous method, this plastic layer is essentially nonoriented other than incidental orientation normally produced during the casting or blowing of a plastic film.

The polymer constituting the central layer is chosen among one of the following thermoplastics: polypropylene, high and low density polyethylenes, polyesters and polyamides. It is interesting to note that, the polymer not being in contact with the food product or the beverage contained within the container, it is possible and recommended to use recycled polymers. Trials have been made with recycled polyesters and polypropylene and give completely satisfactory results.

The metal is either steel, tin plated or not, coated with chrome, zinc, nickel, or of chrome-chrome oxide, or of aluminum or an alloy of aluminum, aluminum alloys being preferred. It is further preferred that the rupture strength of the metal foil when tested alone and in tension be greater than 185 MPₐ.

The selection of the specific materials and the thicknesses of the layers is preferably such that, when the starting sheet is pulled in uniaxial tension, most of the load is borne by the combined metal layers. More preferably, the percentage of the load which is borne by the combined metal layers should be greater than or equal to 70%.

The metal foils can be of different thicknesses or constituted of different metals. One could, for reasons explained later, use a metal foil corresponding to the exterior of the can thicker than that which corresponds to the interior of the can or choose for the foil corresponding to the interior of the can an alloy having a better corrosion resistance and for the foil corresponding to the exterior of the can an alloy having better mechanical strength.

A layer of appropriate adhesive of a thickness between 1 and 20 µm (microns) can be interposed between the central layer of polymer and the foil or foils of metal, the thickness of the adhesive being included in the total thickness of polymer P.

The adhesive interposed between polymer and metal is either a thermoset polymer, for example a polyurethane or an epoxy, or a thermoplastic polymer such as polyolefins modified in a classical fashion by an ethylenic acid (malic, crotonic, etc.) ethylene acrylics (EAA), polyesters or copolymers of the monomers corresponding to the above indicated polymers.

The adherence of the metallic foils to the central polymer layer is evidently an important characteristic of the metal-plastic constructions and of the can bodies produced from these constructions. This adherence is measured by the peel strength, the force necessary for detaching a band of metal foil of determined width from its polymer support and which is expressed, therefore, in force per unit length. The constructions intended for the production of drawn and ironed can bodies ought to have a peel strength higher than 0.4 newtons per millimeter.

The metal-plastic constructions can themselves be coated on one or both sides with a varnish or a polymer film without parting from the framework of the present invention.

Another object of the invention concerns the finished cans prepared starting from the bodies or forms of which the characteristics are indicated above. To fabricate a can starting from a can body, one first proceeds to trim the body to height by shearing the upper part of the walls, then to neck this upper part. The upper edge ought to be then rolled to a small radius of curvature to permit the seaming of the end after filling the can. Because, in the course of this operation of bending the metal-plastic construction according to this small radius, one observes that the metal foil the farther from the center of curvature, that which is in extension, breaks at the point where the radius is the smallest, the other metal foil remaining intact. This phenomenon, for reasons which it would take too long to explain here, does not occur with a homogeneous metal of the same thickness without a polymer layer. Faced with this problem, the inventors have first of all searched for a solution, then have rapidly set forth the hypothesis that this rupture of the metal foil in extension had no effect on the mechanical strength of the can which had been filled and seamed. What could be feared, in effect, is that a can with a rolled flange in which one of the two metal foils is ruptured would not be able to resist the tensile stresses created by the internal pressure which tends to detach the end. However, the internal _stresses in the axial direction of a pressurized cylinder are approximately half of those in the direction perpendicular to the axis. Thus, if there is enough metal in the complete metal-plastic construction, with its two layers of metal, to resist the stresses in a plane perpendicular to the axis, there is enough metal in the remaining intact layer to resist the axial stresses. This hypothesis has been confirmed by calculations. Moreover, the total thickness in the brim is, in general, higher than that of the thinnest part of the wall, which gives a margin of safety. It is also possible for reinforcing the can to choose for the external foil a higher thickness or a stronger alloy than for the internal layer. Finally, the exterior appearance of the can will not be affected since the broken part of the metal foil will be covered by the folded edge of the end in such a way that the final user of the can will not even notice it. A final can of metal-plastic metal-polymer-metal, possessing an upper rolled border in which the metal foil the greater distance from the center of curvature, which is therefore in extension, is ruptured at the location where the radius is the smallest constitutes a second object of the invention.

Besides the technique of seaming, it is equally possible to attach the cover to the metal-plastic can by any other known technique; heat sealing, gluing.

The invention concerns equally a process for fabricating drawn and ironed cans intended for the packaging of beverages characterized in that it includes the following steps:
a) Preparation of a strip of metal-plastic construction including successively a metal layer, a thermoplastic polymer layer, a second metal layer, a layer of polymer adhesive being able to be interposed between each metal layer and the polymer layer.
b) Cutting circular discs from the strip.
c) Drawing the discs to give cups in two successive passes, each of the two passes being made preferably with a cylindrical punch having a circular base in which the generatrice are connected on the base by a radius of curvature between 5 and 10 millimeters and the second pass being made preferably with an entry angle of the fixed platen with the horizontal between 10 degrees and 70 degrees.
d) Ironing of the wall of the cups thus obtained by means of a series of ironing rings preferably 4 in number of which the first, called calibration, diminishes the wall thickness only by between 2 and 25%.

The metal-plastic construction objects of step a of the invention are prepared by different known methods. The most commonly used are direct co-extrusion, thermal sealing, and induction gluing. These last two methods are preferably practiced on a continuous line fed with plastic films and metal strips.

Direct co-extrusion consists of extruding between the two metal foils which are unrolled continuously and which constitute the external layers, the central polymer layer on one side and the others of this central layer the two thin layers of adhesive. The composite product thus obtained passes then between the rollers in order to achieve the adherence between the different layers. This technique evidently applies just in the case of thermoplastic adhesives.

Heat bonding consists in starting with a composite strip of polymers including a central layer of polymer coated on each of its faces by the adhesive layer, here also thermoplastic, and of introducing this strip between two metal foils. The heat bonding is assured by the passage of the composite product thus obtained between two rolls heated to a temperature sufficient to melt or at least soften the adhesive layer sufficiently in a fashion to guarantee the adhesion between the polymer core and the metal foils.

Finally, the gluing by induction consists of coating the inside faces of the two metal foils with a thermosetting adhesive by a known method and applying these foils from one side and the other on the strip of central polymer with the aid of rollers.

The forming of the cans includes a first step c consisting in general of one or several successive drawing passes in using a device such as that represented in Figure 1. In order to adapt the operating conditions to the particular case of metal-plastic constructions of the MPM type, the inventors have been led to prefer one particular shape of punch base and of entry shape of the die plate which work together to assure a drawing of the construction without forming cracks, wrinkles or delaminations.

The punch, of a general shape of a cylinder of revolution, presents, according to one of the preferred methods of the invention, an axial section of which the generatrice are connected at the base of the punch by a circular arc of a radius between 5 and 10 mm. This connection can be done directly on the base of the punch or by an intermediary, seen in section of a second circular arc of which the center lies on the axis of revolution of the punch. Figures 5a and 5b illustrate the two variations indicated above.

Figure 5a represents the simplest shape of the embodiment. The punch 9 is viewed in section through the axis; it takes the shape of a cylinder of revolution about the axis 10. The generatrix 11 is connected to the base by a circular arc of radius R1 which falls between 5 and 10 mm (8 mm for example for punch with a diameter of 85 mm). This circular arc generates by revolution a portion of a torus.

Figure 5b represents a developed shape a little more complicated; the generatrice are joined on the base by a first circular arc 14 of radius R1 between 5 and 10 mm which connects tangentially to a second circular arc of large radius R2 (15) centered on the axis of the punch. The circular arc (15) generates a spherical dome and the circular arc (14) a portion of a torus. By way of example, R1 could be in the order of 6 mm and R2 in the order of 250 mm.

The other preferred method of the invention, cooperating with the particular shape of the punch described above, is the shape, also particular, of the entry of the die plate utilized for the second drawing pass. Normally, drawing die plates have the shape represented schematically in Figure la which represents the first drawing pass starting from a flat circular disc as has been explained above. Figure 6 represents the following drawing passes according to the invention of which the starting material is no longer a disc but a shape already drawn during the course of the first pass. The cup (24) is in the process of drawing, its initial diameter corresponding to the upper part (25) is in the process of reduction towards its final diameter (26) defined by the space between the punch (27) and the die plate (28). Correspondingly, the height of the walls grows without that there be an ironing in the normal sense of the word, that is a significant reduction of the thickness. An inside pressure plate (29) is positioned at the interior of the starting cup.

The inventors have found that the angle at which the generatrix of the entry cone makes with the horizontal plane perpendicular to the axis of the punch is critical for drawing metal-plastic constructions of type MPM. This angle ought to be between 10 degrees and 70 degrees and preferably around 60 degrees.

The forming of cans includes a last step (d), consisting of an ironing operation permitting the elongation of the wall with a corresponding thinning of the wall. This operation is represented schematically in Figure 2.

The applicant has discovered that it was possible to iron the walls of a cup drawn from an MPM disc without engendering flaws such as cracks and delaminations, preferably by processing in four successive ironing passes instead of the three generally practiced in particular according to the teaching in European Patent Application EP 0402006. More preferred still, the first of these successive passes is a simple calibrating pass with a rate of thickness reduction between 2 and 25%.

The examples which follow illustrate, on particular cases, the different steps of the invention.

### Example 1

A strip of polypropylene of 300 µm (microns) thickness has been coated on each of its faces with a layer of 10 µm (microns) in thickness of an adhesive consisting of a film of maleic acid modified polypropylene. The two films of adhesive have been applied on the film cold by passing between two rolls. The composite strip thus obtained has been then introduced continuously between two foils of 100 µm (micron) thick aluminum alloy 3003, a manganese alloy according to the standards of the "Aluminum Association", each unwound from a bobbin and preheated by passage through an oven at a temperature of 200°C in a fashion to melt the adhesive. The MPM construction obtained was then passed between the rollers exerting a pressure of around 4000 kPa, then rolled onto a bobbin. Starting from this construction, circular discs of 140 mm in diameter were cut out. These discs have been then drawn in two successive passes with the aid of a punch analogous to that represented in figure 5a with R1 = 8 mm. For the second drawing pass, a die plate for which the angle alpha was 60° has been used. The first pass has given cups with an outside diameter of 86 mm and a height of 35 mm. The second pass has given cups with an outside diameter of 67 mm and a height of 56 mm. These cylindrical cups carried by a punch have finally been ironed by passage through a tool including a series of four rings of successively smaller diameters to give cups of beverage cans of 66 mm in diameter and 130 mm in height. The respective reductions in wall thickness express in % of the initial thickness are the following: 20%, 40%, 52% and 57%. Careful examination of these cups have not shown evidence of any cracks of the metal or of the plastic. No delamination between the metal and the plastic has been observed.

### Example 2

A composite MPM strip has been prepared by coextruding between two foils of the same 3003 alloy as in Example 1, but of a thickness of 80 µm (microns), a core comprised of polypropylene in 250 µm (microns) of thickness and on one side and the others of this core a layer of adhesive comprised of maleic acid modified polypropylene of 10 µm (microns) in thickness. The adhesion has been achieved by passage between two rolls heated to 200°C, while applying a pressure of 4000 kPa. Some beverage bottle cups have been fabricated under the same conditions as in Example 1. The examination of these cups has shown no cracking of the metal or of the plastic. No delamination between the metal and the plastic has been observed.

### Example 3

An MPM composite strip has been prepared by coextrusion under the same conditions and with the same component as those in Example 2, but in using for the core polypropylene recycled from cans fabricated with this same MPM construction. Even though the recovery of the polypropylene from the used cans did not permit the separation of the adhesive from the polymer, the constructions obtained were of excellent quality and did not show either cracks or delamination. Beverage can cups have been produced under the same conditions as for Example 1. The examination of these cups has not exhibited any cracks of the metal or of the plastic. No delamination between the metal and the plastic has been observed.

### Example 4

Under the same operational conditions as those of Example 2, a MPM construction has been fabricated comprising successively: a foil of 3003 alloy of 80 µm (microns) in thickness, a layer of adhesive of amorphous polyethylene terephtalate of 10 µm (microns) in thickness, a layer of polyethylene terephtalate of 200 µm (microns) in thickness, another layer of amorphous polyethylene terephtalate of 10 µm (microns) of thickness, finally another foil of 3003 alloy of 80 µm (microns) in thickness. The beverage can cups have been fabricated under the same conditions as in Example 1. The examination of these cups has not shown any cracks of the metal or of the plastic. No delamination between the metal and the plastic has been observed.

### Example 5

Example 5 concerns the same fabrication of cups as in Example 4, with the comparative difference that the polyethylene terephtalate used came from the recovery of used plastic bottles. These bottles, after washing and drying, have been ground and have been introduced in the feed hopper of the extruder. No quality problem has been observed either on the construction or on the cups obtained by drawing and ironing.

## Claims

1. A drawn and ironed can body comprising a base and an upstanding sidewall, the base and the sidewall having an Mᵢ-P-Mₑ type laminar construction, wherein Mᵢ and Mₑ are inner and outer metal foil layers, respectively, and P is central polymer layer and the ratio of the thicknesses P/(Mᵢ and Mₑ) is greater than 0.5, and the thickness of the sidewall being thinner than the thickness of the base.

2. A can body according to Claim 1, characterized in that the central polymer layer is essentially nonoriented.

3. A can body according to Claim 1 or 2, characterized in that the thickness of the polymer layer P is between 100 and 500 µm and the thickness of each of the metal layers Mᵢ and Mₑ is between 25 and 150 µm.

4. A can body according to any one of Claims 1 to 3, characterized in that the peel strength of the metal layers to plastic layers in the laminar construction is greater than 0.4 N/mm.

5. A can body according to any one of Claims 1 to 4, wherein Mᵢ and Mₑ are metal foils independently selected from foils of steel, tin-plated steel, steel coated with chrome, zinc or nickel, chrome-chrome oxide coated aluminum and aluminum alloys.

6. A can body according to any one of Claims 1 to 5, wherein polymer layer P comprises a thermoplastic polymer selected from the group consisting of polypropylene, high density polyethylene, low density polyethylene, polyesters, and nylon.

7. A can body according to any one of Claims 1 to 6, further comprising a layer of adhesive having a thickness between 1 and 20 microns interposed between the central polymer layer P and each of the foil layers Mᵢ and Mₑ, the thickness of adhesive being included in the total thickness of polymer P.

8. A can body according to any one of Claims 1 to 7, wherein the sidewall portions includes an upper rolled region in which the metal foil Mᵢ is in extension and is ruptured at the location where the radius of curvature is the smallest.

9. A can body according to any one of Claims 1 to 8, characterized in that the metal foil Mₑ forming on outside surface of the can body is thicker than foil layer Mᵢ forming on inside of the can body.

10. A method for making can bodies having reduced metal content, said method comprising:
providing a sheet of an Mᵢ-P-Mₑ laminate, wherein Mᵢ and Mₑ are inner and outer metal foil layers, respectively, and P is a central polymer layer and the ratio of the thicknesses P/(Mᵢ + Mₑ) is greater than 0.5;
cutting discs (1) from the sheet;
drawing the discs in at least one drawing pass to form a cup (5, 24);
ironing the cup in at least one ironing pass to form a can body including a base portion and an upstanding sidewall portion (25), the upstanding sidewall portion having an overall thickness less than the base portion.

11. A method as in Claim 10, wherein in the laminate sheet, the central polymer layer P has a thickness of between 100 and 500 µm and each of the metal foils Mᵢ and Mₑ independently has a thickness of between 25 and 150 µm.

## Patentansprüche

1. Gezogener und abstreckgezogener Dosenkörper, der eine Basis und eine aufrechte Seitenwand umfasst, wobei die Basis und die Seitenwand einen Mᵢ-P-Mₑ-artig geschichteten Aufbau aufweisen, wobei Mᵢ und Mₑ jeweils innere und äussere Metallfolienschichten sind und P eine zentrale Polymerschicht ist, und das Verhältnis der Dicken P/(Mᵢ und Mₑ) grösser ist als 0,5 und die Dicke von der Seitenwand geringer als die Dicke der von der Basis ist.

2. Dosenkörper gemäß Anspruch 1, dadurch gekennzeichnet, dass die zentrale Polymerschicht im Wesentlichen nicht orientiert ist.

3. Dosenkörper gemäß Anspruch 1 oder 2, dadurch gekennzeichnet, dass die Dicke der zentralen Polymerschicht P zwischen 100 und 500 µm ist und die Dicke jeder der Metallschichten Mᵢ und Mₑ zwischen 25 und 150 µm ist.

4. Dosenkörper gemäß einem der Ansprüche 1 bis 3, dadurch gekennzeichnet, dass der Abziehwiderstand der Metallschichten gegen die Kunststoffschichten in dem geschichteten Aufbau größer als 0,4 N/mm ist.

5. Dosenkörper gemäß einem Der Ansprüche 1 bis 4, wobei Mᵢ und Mₑ Metallfolien sind, die unabhängig ausgewählt sind aus Folien aus Stahl, verzinntem Stahl, mit Chrom, Zink oder Nickel beschichtetem Stahl, Chrom-Chromoxid beschichtetem Aluminium und Aluminiumlegierungen.

6. Dosenkörper gemäß einem der Ansprüche 1 bis 5, wobei die Polymerschicht P ein thermoplastisches Polymer umfasst, ausgewählt aus der Gruppe bestehend aus Polypropylen, Niederdruckpolyethylen, Hochdruckpolyethylen, Polyestern und Nylon.

7. Dosenkörper gemäß einem der Ansprüche 1 bis 6, der weiter eine Haftmittelschicht mit einer Dicke zwischen 1 und 20 µm umfasst, die zwischen der zentralen Polymerschicht P und jeder der Folienschichten Mᵢ und Mₑ eingefügt ist, wobei die Dicke des Haftmittels in der Gesamtdicke der Polymerschicht P enthalten ist.

8. Dosenkörper gemäß einem der Ansprüche 1 bis 7, wobei die Seitenwandabschnitte einen oberen gerollten Bereich aufweisen, in dem die Metallfolie Mᵢ gedehnt ist und an dem Ort zerrissen ist, an dem der Krümmungsradius am kleinsten ist.

9. Dosenkörper gemäß einem der Ansprüche 1 bis 8, dadurch gekennzeichnet, dass die Metallfolie Mₑ, die eine äussere Oberfläche des Dosenkörpers bildet, dicker ist als Folienschicht Mᵢ, die ein Inneres des Dosenkörpers bildet.

10. Verfahren zum Herstellen von Dosenkörpern mit verringertem Metallgehalt, wobei das Verfahren umfasst:
bereitstellen eines Bogens eines Mᵢ-P-Mₑ-Laminates, wobei Mᵢ und Mₑ jeweils innere und äussere Metallfolienschichten sind und P eine zentrale Polymerschicht ist und wobei das Verhältnis der Dicken P/(Mᵢ und Mₑ) grösser als 0,5 ist;
schneiden von Scheiben (1) aus dem Bogen;
ziehen der Scheiben in wenigstens einem Zieh-Arbeitsgang um einen Napf (5, 24) zu formen; abstreckziehen des Napfes in wenigstens einem Abstreck-Arbeitsgang um einen Dosenkörper zu formen, der einen Basisabschnitt und einen aufrechten Seitenwandabschnitt (25) umfasst, wobei der aufrechte Seitenwandabschnitt eine geringere Gesamtdicke als der Basisabschnitt aufweist.

11. Ein Verfahren nach Anspruch 10, wobei in dem Laminat Bogen die Polymerschicht P eine Dicke zwischen 100 und 500 µm aufweist und jede der Metallfolien Mᵢ und Mₑ unabhängig eine Dicke zwischen 25 und 150 µm aufweist.

## Revendications

1. Corps de boîte embouti et étiré comprenant une base et une paroi latérale dressée, la base et la paroi latérale présentant une construction laminaire de type Mᵢ-P-M_{c}, dans laquelle Mᵢ et M_{c} sont des couches de feuilles métalliques intérieure et extérieure, respectivement et P est une couche centrale de polymère et le rapport des épaisseurs P/(Mᵢ et M_{c}) est supérieur à 0,5, et l'épaisseur de la paroi latérale étant plus mince que l'épaisseur de la base.

2. Corps de boîte selon la revendication 1, caractérisé en ce que la couche centrale de polymère est essentiellement non orientée.

3. Corps de boîte selon la revendication 1 ou 2, caractérisé en ce que l'épaisseur de la couche de polymère P est entre 100 et 500 µm et l'épaisseur de chacune des couches métalliques Mᵢ et M_{c} est entre 25 et 150 µm.

4. Corps de boîte selon l'une quelconque des revendications 1 à 3, caractérisé en ce que la résistance à l'écaillage des couches métalliques sur les couches en matière plastique dans la construction laminaire est supérieure à 0,4 N/mm.

5. Corps de boîte selon l'une quelconque des revendications 1 à 4, dans lequel Mᵢ et M_{c} sont des feuilles métalliques choisies indépendamment à partir de feuilles d'acier, d'acier étamé, d'acier revêtu de chrome, de zinc ou de nickel, de l'aluminium revêtu de chrome-oxyde de chrome et des alliages d'aluminium.

6. Corps de boîte selon l'une quelconques des revendications 1 à 5, dans lequel la couche de polymère P comprend un polymère thermoplastique choisi à partir du groupe constitué du polypropylène, du polyéthylène à haute densité, du polyéthylène à basse densité, des polyesters, et du nylon.

7. Corps de boîte selon l'une quelconque des revendications 1 à 6, comprenant en outre une couche d'adhésif présentant une épaisseur entre 1 et 20 micromètres intercalée entre la couche de polymère centrale P et chacune des couches de feuilles Mᵢ et M_{c}, l'épaisseur de l'adhésif étant incluse dans l'épaisseur totale du polymère P.

8. Corps de boîte selon l'une quelconque des revendications 1 à 7, dans lequel les parties de paroi latérales comprennent une région laminée supérieure dans laquelle la feuille métallique Mᵢ est en extension et est rompue à l'emplacement où le rayon de courbure est le plus petit.

9. Corps de boîte selon l'une quelconque des revendications 1 à 8, caractérisé en ce que la feuille métallique M_{c} formant une surface extérieure du corps de boîte est plus épaisse que la couche de feuille Mᵢ formant la surface intérieure du corps de boîte.

10. Procédé destiné à réaliser des corps de boîte présentant une teneur en métal réduite, ledit procédé comprenant :
la fourniture d'une feuille stratifiée Mᵢ-P-M_{c}, dans laquelle Mᵢ et M_{c} sont des couches de feuilles métalliques intérieure et extérieure, respectivement et P est une couche de polymère centrale et le rapport des épaisseurs P/(Mᵢ+M_{c}) est supérieur à 0,5,
découper des disques (1) à partir de la feuille,
emboutir les disques dans au moins une passe d'emboutissage pour former une coupelle (5, 24),
étirer la coupelle en au moins une passe d'étirage pour former un corps de boîte comprenant une partie de base et une partie de paroi latérale dressée (25), la partie de paroi latérale dressée présentant une épaisseur globale inférieure à la partie de base.

11. Procédé selon la revendication 10, dans lequel dans la feuille de stratifié, la couche de polymère centrale P présente une épaisseur entre 100 et 500 µm et chacune des feuilles métalliques Mᵢ et M_{c} présente indépendamment une épaisseur entre 25 et 150 µm.
